

Sept. 22, 1936.

E. HURST

2,055,411

FIBROUS MATERIAL AND METHOD OF MAKING THE SAME

Filed April 28, 1934



INVENTOR.  
*Edward Hurst*  
BY  
*Gifford, Scull & Burgess*  
ATTORNEYS.

## UNITED STATES PATENT OFFICE

2,055,411

FIBROUS MATERIAL AND METHOD OF  
MAKING THE SAME

Edward Hurst, West Newton, Mass., assignor to  
United Cotton Products Company, Fall River,  
Mass., a corporation of Massachusetts

Application April 28, 1934, Serial No. 722,868

10 Claims. (Cl. 19—155)

This invention relates to a novel and improved form of fibrous material and method of making the same, the novel features of which will be best understood from the following description 5 and the annexed drawing, in which I have shown a selected embodiment of the invention and in which:

Fig. 1 is a vertical sectional diagrammatic view of an apparatus which may be used in the 10 practice of this invention;

Fig. 2 is a fragmentary view on an enlarged scale of part of Fig. 1;

Fig. 3 is a perspective view of a small part of the web before impregnating;

Fig. 4 is a view on an enlarged scale illustrating diagrammatically how the different membranes come together.

The invention of this application is an improvement upon certain features disclosed in the 20 copending application of myself and Myrick Crane, Ser. No. 673,392. In that application and in a division thereof we have disclosed and claimed the general combination shown in Fig. 1 of the drawing of this application, together with 25 the method of operating the same and the resulting product.

As more fully set forth in that application, the invention may be practiced by forming a plurality of what may conveniently be termed 30 membranes, on cards 1, these cards being of any suitable or usual form. Each of these cards is provided with the usual doffer 2 and comb 3 adapted to remove the membrane, or lap, as it is sometimes called, from the doffer. The membranes 4, 5, 6, and 7 coming from the respective cards are passed through orifices 8 in the floor 9 on to a conveyor 10 which may be vibrated as described in said copending application, to aid in causing an interlocking of the fibers of 40 the respective membranes, to form what may conveniently be termed a web 11, which may be passed between rolls 12 and then to the impregnating rolls 13 associated with the vat 14. The impregnated web may then be dried upon 45 a festoon drier 15. The material used may be cotton or any other unspun fibrous material found to be suitable.

In the practice of the invention as described and claimed in the aforesaid copending application, I have found that improved results are 50 achieved by the method which I shall now describe. Referring particularly to Fig. 2, it will be seen that the membrane, which in this figure is shown as the membrane 4, is taken by the 55 comb 3 from the doffer 2 as described above.

It is well known that such a membrane of unspun fibers, as the comb removes it from the doffer of a card, is extremely light and filmy, and this is particularly true with cotton fibers to which I have found that my invention is particularly adaptable. The fibers of cotton, as is well known, are kinky in the natural state, and this kinkiness is removed to some extent during the carding process, this carding resulting in the arrangement of the fibers in the lap or membrane approximately parallel to each other and extending in a direction longitudinally of the membrane. The membrane formed of these fibers is extremely weak, as is well known.

I have discovered that I can so treat such 15 membrane that its strength will be substantially increased and so that the fibers therein will be interlocked and interwoven with each other in a multiplicity of planes. At the same time, the membrane is so processed that it will easily combine with other membranes when placed in contact therewith, and which have been similarly processed.

The above results are achieved by what I may conveniently term aerodynamic weaving. One 25 method of operation can be best understood from Fig. 2, where the membrane 4 is shown as coming from the card 3 and passing through one of the orifices 8 in the floor 9. Extending upwardly from the rear wall 16 of the orifice is 30 a wall 17 having a smooth surface adjacent the membrane, and extending upwardly from the opposite wall 18 of the orifice is a second wall 19 likewise having a smooth surface facing the membrane and extending up above the comb 3. 35

The membrane, after leaving the doffer, is caused to pass downwardly between the walls 17 and 19 and through the orifice on to the conveyor.

The walls 17 and 19 form parts of an enclosure in which the air pressure is less than that beneath 40 the floor 9. In this connection, it might be said that the conveyor itself is enclosed to a sufficient extent to prevent disturbance, by uncontrolled currents of air, of the membranes before they reach the conveyor or of the web formed of the 45 membranes, although it is deemed unnecessary to show the enclosing means in the drawing. The differential in pressure between the air beneath the floor 9 and that between the walls 17 and 19 is, of course, a slight one, because of the 50 delicacy of the material being handled, but nevertheless it is a positive one and one which is carefully controlled to get the desired results.

The walls of the orifice 8 are preferably stream-lined in some such manner as indicated, so as to 55



without substantially disturbing said continuity, and passing said membrane along a walled conduit.

2. The method of forming a web which comprises forming a membrane of unspun fibers, passing currents of air along opposite sides of said membrane, preventing turbulence in said currents sufficiently to maintain the continuity of the membrane, causing some of said air to flow through the membrane with sufficient force to change the relation of the fibers therein to each other without substantially disturbing said continuity, passing said membrane along a walled conduit, and causing the currents of air an opposite sides of the membrane to maintain it out of contact with the walls of the conduit.

3. The method of forming a web which comprises forming a membrane of unspun fibers, passing said membrane along a current of air traveling in a direction opposite to the direction of movement of the membrane, and causing said air to pass through said membrane, said air being under a pressure which is sufficient in amount to change the positions of the individual fibers relative to each other and thus to cause them to interlock with each other, but is insufficient to substantially disturb the continuity of the membrane.

4. The method of forming a web which comprises forming a membrane of unspun fibers, passing currents of air along opposite sides of said membrane, maintaining a differential of pressure between opposite sides of the membrane to cause some of the air to flow therethrough, said differential being sufficient in amount to change the positions of the individual fibers relative to each other and thus to cause them to interlock with each other, but being insufficient to substantially disturb the continuity of the membrane.

5. The method of forming a web which comprises forming a membrane of unspun fibers, passing currents of air along opposite sides of said membrane, maintaining a differential of pressure between opposite sides of the membrane to cause some of the air to flow therethrough, said differential being sufficient in amount to change the positions of the individual fibers relative to each other and thus to cause them to interlock with each other, but insufficient to substantially disturb the continuity of the membrane, and preventing turbulence in said air sufficient to disturb said continuity.

6. The method of forming a web which comprises carding unspun fibers to form a membrane, passing said membrane along a walled conduit and through an orifice against currents of air flowing through said orifice and along said conduit on opposite sides of the membrane, maintaining a differential of pressure between opposite

sides of the membrane to cause some of the air to flow therethrough, said differential being sufficient in amount to change the positions of the individual fibers relative to each other and thus to cause them to interlock with each other, but is insufficient to substantially disturb the continuity of the membrane.

7. The method of forming a web which comprises carding unspun fibers to form a membrane, passing said membrane along a walled conduit and through an orifice against currents of air flowing through said orifice and along said conduit on opposite sides of the membrane, maintaining a differential of pressure between opposite sides of the membrane to cause some of the air to flow therethrough, said differential being sufficient in amount to change the positions of the individual fibers relative to each other and thus to cause them to interlock with each other, but is insufficient to substantially disturb the continuity of the membrane, and preventing turbulence in said air sufficient to disturb said continuity.

8. The method of forming a web which comprises carding upspun fibers to form a membrane, passing said membrane along a walled conduit and through an orifice while maintaining it substantially out of contact with the walls of said conduit and orifice, and directing a current of air into contact with said fibers under a pressure which is sufficient in amount to change the positions of the individual fibers relative to each other and thus to cause them to interlock with each other, but is insufficient to substantially disturb the continuity of the membrane.

9. The method of forming a web which comprises forming a membrane of unspun fibers, maintaining a differential of pressure between opposite sides of the membrane to cause a current of air to flow therethrough, said differential being sufficiently high in amount to change the positions of individual fibers within the membrane, relatively to each other, and thus to cause said fibers to interlock with each other, but being sufficiently low in amount to avoid substantial disturbance of the continuity of the membrane.

10. The method of forming a web which comprises forming a membrane of unspun fibers, passing said membrane through an orifice, and maintaining within said orifice a differential of pressure between opposite sides of the membrane to cause a current of air to flow therethrough, said differential being sufficiently high in amount to change the positions of individual fibers within the membrane, relatively to each other, and thus to cause said fibers to interlock with each other, but being sufficiently low in amount to avoid substantial disturbance of the continuity of the membrane.

EDWARD HURST. 60